

United States Patent  
Gitlesen

[15] 3,653,880  
[45] Apr. 4, 1972

[54] MAGNESIUM CAST ALLOYS WITH  
LITTLE TENDENCY TO HOT-CRACK

1,942,041 1/1934 Wood..... 75/168 B  
1,975,375 10/1934 Schichtel..... 75/168 D  
1,975,376 10/1934 Schichtel..... 75/168 D  
2,000,115 5/1935 Wood..... 75/168 C  
2,041,866 5/1936 Schichtel..... 75/168 C  
2,041,867 5/1936 Schichtel..... 75/168

[72] Inventor: Gunnar Gitlesen, Porsgrunn, Norway

[73] Assignee: Norsk Hydro A/S, Oslo, Norway

[22] Filed: Jan. 8, 1970

[21] Appl. No.: 1,449

[52] U.S. Cl..... 75/168 C, 75/168 R, 75/168 B,  
148/32

[51] Int. Cl..... C22c 23/00

[58] Field of Search..... 75/168; 148/32

[56] References Cited

UNITED STATES PATENTS

2,094,332 9/1937 Schichtel et al..... 75/168 C

Primary Examiner—Charles N. Lovell  
Attorney—Wenderoth, Lind & Ponack

[57] ABSTRACT

Magnesium cast alloys containing 3-10 percent aluminum, 0.3-2 percent zinc and 0.1-0.4 percent bismuth or tin, all by weight, showing little tendency to hot-crack.

4 Claims, 1 Drawing Figure



Patented April 4, 1972

3,653,880



GUNNAR GITLESEN,

INVENTOR

BY *Wendell Lind-Praas*

ATTORNEY

**MAGNESIUM CAST ALLOYS WITH LITTLE TENDENCY  
TO HOT-CRACK**

The invention relates to an aluminium-containing magnesium cast alloy with little tendency to hot-crack.

Magnesium alloys containing 3 to 10 percent of aluminium and usually 0.3 to 2 percent of zinc, for instance AZ 91, have several good properties when used for casting purposes, of which may be mentioned adequate fluidity (Formfullvermogen), die castability and also satisfactory mechanical properties at temperatures up to about 100°C.

These alloys are not particularly liable to hot-crack, but their field of application would be even wider if the tendency to hot-crack could be further reduced, as a modern technique of pressure die casting provides possibilities for mass production of a growing variety of cast articles, including articles of such a design and shape as to increase the liability to hot-crack, thus requiring an alloy which per se has little tendency to hot-crack.

Hot-crack may occur in castings in the solid-liquid interface during the process of cooling.

The above-mentioned type of cast alloys have a considerable temperature range of solidification, and consequently stress conditions more easily arise in the casting during solidification, for instance due to hindered contraction occurring when the casting mould and/or the core prevent the free contraction of the casting, and also due to contraction distortion in the casting itself. The tendency to hot-crack is increased when the various portions of the casting are not cooled at the same rate, which will readily occur when the casting is not of a fairly uniform thickness.

Different ways and means are known to counteract the tendency of cast alloys to hot-crack. As to magnesium alloys of the above-mentioned type, it is known that variation of the aluminium and zinc content has an influence on the alloy's tendency to hot-crack.

Surprisingly it was found that adding bismuth to magnesium alloys of the above mentioned type has a very marked effect in reducing the hot-crack tendency of the alloy. Tin was also found to have a favorable effect, although not as strong an effect as bismuth.

The actual proportions of bismuth or tin used in practice are below 1 %. The experiments carried out show a maximum effect at 0.1 to 0.4 percent by weight of bismuth. The maximum effect of tin is also found to be between 0.1 to 0.4 percent by weight, although the effect in this case is, as mentioned above, somewhat smaller. To the alloy can be added, if desired, up to about 0.5 percent of manganese, up to about 0.5 percent of silicon, up to about 0.5 percent of copper, and the usual quantities of metal to inhibit burning or oxidation, such as beryllium.

In the following some illustrating experiments will be described:

A. 1. There was made an alloy of AZ 91 type (9 % aluminium, 0.7 percent zinc and 0.2 percent manganese) containing varying quantities of bismuth and tin respectively. The following table shows the content of bismuth and tin:

| % by weight of bismuth | % by weight of tin |
|------------------------|--------------------|
| 0                      | 0                  |
| 0.10                   | 0.11               |

|      |      |
|------|------|
| 0.20 | 0.30 |
| 0.35 | 0.31 |
| 0.40 | 0.50 |
| 0.50 |      |

5 These alloys were treated as to hot-crack in a modified permanent mould of the type described in "Giesserei," 45, Heft 26 (1958), p.761-765.

The results will appear from the graph. The ordinate represents the temperature deviation in degrees centigrade from the critical temperature for AZ 91 without bismuth or tin. The term "critical temperature" as used herein means the lowest mould temperature that gives a crackfree test ingot. The curve for bismuth shows a temperature deviation of 70° to 80° C. for an addition of bismuth of 0.2 to 0.3 percent. This is 10 a very great difference in temperature, which means that the favorable effect of an addition of 0.2 to 0.3 percent of bismuth to the alloy is considerable.

The graph further shows a similar effect with tin of 30° to 40° C. between 0.1 and 0.4 percent by weight of tin. The tin 15 content may be within the range 0.2 to 0.3 percent by weight.

2. An addition of 0.3 percent of bismuth to an AZ 61 alloy (6 % of aluminium, 0.7 percent of zinc, 0.2 percent manganese) gave an improvement of 55° C. compared with AZ 61 without bismuth in experiments with the above-mentioned 20 mould.

The alloys under 1) and 2) showed a tensile strength normal 25 for AZ 91 alloys. Further experiments showed that the addition of bismuth did not give increased tendency to corrosion as tested by dipping in a 3 percent NaCl solution.

30 B. AZ 91 alloys with and without bismuth were pressure die cast to a special hot-crack sensitive place. The tendency to hot-crack was examined in the cast pieces.

Result:

AZ 91: 4 cracks per piece (average for 200 pieces) 3 percent entirely faultless pieces

AZ 91 with 0.3 percent Bi: 3.3 cracks per piece (average for 100 pieces) 7 percent entirely faultless pieces

It is evident from the above experiments that the hot-crack 35 tendency in aluminium-containing magnesium alloys can be prevented to a large extent by addition of bismuth or tin, particularly bismuth.

The aluminium content of the alloys of this invention may be 40 3-10 percent by weight for tin-containing alloys and 5.5-10 percent by weight, including the narrower range of 7.5-10 percent, for bismuth-containing alloys.

I claim:

1. Magnesium cast alloy consisting essentially of 3 to 10 percent by weight of aluminium, 0.3 to 2 percent by weight of zinc and 0.1 to 0.4 percent by weight of bismuth or tin, balance 45 magnesium with the proviso that the aluminium content of the alloy containing bismuth is 5.5 to 10 percent by weight, said alloy having a reduced tendency to hot-crack.

2. The alloy according to claim 1, containing bismuth, wherein the aluminium content is from 7.5 to 10 percent by weight.

3. The alloy according to claim 1, wherein the content of bismuth or tin is 0.2 to 0.3 percent by weight.

4. The alloy according to claim 4, containing up to 0.5 percent by weight of manganese, up to 0.5 percent by weight of silicon and up to 0.5 percent by weight of copper.

\* \* \* \* \*